

# UNITED STATES PATENT OFFICE.

WILLIAM D. BERRY, OF NEW BRIGHTON, PENNSYLVANIA.

## BEARING ALLOY.

1,286,921.

Specification of Letters Patent. Patented Dec. 10, 1918.

No Drawing.

Application filed August 13, 1918. Serial No. 249,685.

*To all whom it may concern:*

Be it known that I, WILLIAM D. BERRY, residing at New Brighton, in the county of Beaver and State of Pennsylvania, a citizen 5 of the United States, have invented or discovered a certain new and useful Improvement in Bearing Alloys, of which improvement the following is a specification.

The object of my invention is to provide 10 an alloy for journal bearings for railway car and locomotive axles, rolling-mill roll axles, and in general for axles for all classes of machinery, which alloy will for its intended purpose be in every respect equal 15 to the well known copper-tin-lead alloys, but which will contain no tin and hence may be manufactured considerably cheaper than the usual alloys for bearings, the tin being accordingly conserved for other purposes.

20 My invention is predicated upon my discovery that, within the relative proportions hereinafter specified, antimony may be combined with copper and lead to form a bearing alloy having the same desirable characteristics as the well known copper-tin-lead bearing alloys. To these three elements phosphorus may be, and preferably is, added in small proportions as a hardening agent.

The alloy which I provide is essentially 30 a copper base alloy, the percentages of copper and lead depending somewhat upon the requirements for particular service conditions. Specifically, the alloy may contain from about 60% to 85% copper, from about 1% to 36% lead, and, depending upon the degree of hardness required, from about 3% to 20% antimony. As an additional hardening agent, and also as a deoxidizer, from about .25 to 3% phosphorus may be added

to the alloy. If desired, small quantities of 40 nickel, manganese, silicon or magnesium may be added as a deoxidizing agent or agents.

While, in its broader aspects, my invention is unlimited to an alloy of any specific 45 mix within the above stated limits, I have found an exceptionally desirable alloy to be one comprising about 79% copper, 14% lead, 6% antimony and 1% phosphorus.

In making the alloy, the copper may be 50 first melted in a crucible in the usual manner, and thereafter the phosphorus, antimony, and lead may be successively added in the same manner in which alloying metals are usually added to obtain the most 55 thorough mixing and alloying of the several elements.

The bearing alloy which I provide is, as already stated, a copper base alloy in which 60 tin is entirely displaced by relatively large proportions of antimony.

I claim as my invention:

1. A copper base bearing alloy containing from about 60% to 85% copper, 1% to 35% lead, and 3% to 20% antimony. 65

2. A copper base bearing alloy consisting of from about 60% to 85% copper, 1% to 35% lead, 3% to 20% antimony and .25% to 3% phosphorus.

3. A copper base bearing alloy consisting 70 of about 79% copper, 14% lead, 6% antimony and 1% phosphorus.

In testimony whereof I have hereunto set my hand:

WILLIAM D. BERRY.

Witnesses:

ELMER C. BURKHART,  
W. V. BERRY.